



US007309556B2

(12) **United States Patent**  
**Mc Dougall et al.**

(10) **Patent No.:** **US 7,309,556 B2**  
(45) **Date of Patent:** **\*Dec. 18, 2007**

(54) **BLACK TONER AND DEVELOPER**

(75) Inventors: **Maria N. V. Mc Dougall**, Burlington (CA); **Richard P. N. Veregin**, Mississauga (CA); **Vladislav Skorokhod**, Mississauga (CA); **Mary L. Mc Stravick**, Fairport, NY (US); **Deepak R. Maniar**, Webster, NY (US); **Paul W. Morehouse, Jr.**, Webster, NY (US); **Rachael L. Mc Grath**, Churchville, NY (US); **Jackie Parker**, Mississauga (CA); **Shigang Qui**, Toronto (CA); **Mary B. Schlitzer**, Rochester, NY (US); **Michael D. Thompson**, Rochester, NY (US); **Christopher M. Pattison**, Rochester, NY (US); **Thomas C. Dombroski**, Rochester, NY (US)

(73) Assignee: **Xerox Corporation**, Norwalk, CT (US)

(\*) Notice: Subject to any disclaimer, the term of this patent is extended or adjusted under 35 U.S.C. 154(b) by 368 days.

This patent is subject to a terminal disclaimer.

(21) Appl. No.: **11/083,934**

(22) Filed: **Mar. 21, 2005**

(65) **Prior Publication Data**

US 2005/0250031 A1 Nov. 10, 2005

**Related U.S. Application Data**

(63) Continuation-in-part of application No. 10/839,293, filed on May 6, 2004, now Pat. No. 7,157,200.

(51) **Int. Cl.**  
**G03G 9/087** (2006.01)

(52) **U.S. Cl.** ..... **430/108.6; 430/108.7;**  
430/111.41; 399/267

(58) **Field of Classification Search** ..... 430/108.6,  
430/109.3, 108.7, 111.41; 399/267  
See application file for complete search history.

(56) **References Cited**

**U.S. PATENT DOCUMENTS**

3,981,272 A 9/1976 Smith et al.

|                |         |                                   |
|----------------|---------|-----------------------------------|
| 4,155,329 A    | 5/1979  | Tsukamoto et al.                  |
| 4,375,673 A    | 3/1983  | Lewis et al.                      |
| 4,465,730 A    | 8/1984  | Okada                             |
| 5,236,629 A    | 8/1993  | Mahabadi et al.                   |
| 5,345,298 A    | 9/1994  | Corrigan, Jr.                     |
| 5,416,566 A    | 5/1995  | Edmunds et al.                    |
| 5,545,501 A    | 8/1996  | Tavernier et al.                  |
| 5,847,030 A    | 12/1998 | Mahabadi et al.                   |
| 6,120,967 A    | 9/2000  | Hopper et al.                     |
| 6,319,647 B1   | 11/2001 | Gutman et al.                     |
| 6,361,915 B1   | 3/2002  | Van Dusen et al.                  |
| 6,416,916 B1   | 7/2002  | Silence et al.                    |
| 7,157,200 B2 * | 1/2007  | Mc Stravick et al. .... 430/108.6 |

\* cited by examiner

*Primary Examiner*—John L Goodrow

(74) *Attorney, Agent, or Firm*—Oliff & Berridge PLC

(57) **ABSTRACT**

A developer includes black toner particles and carrier particles, the black toner particles including at least one binder, at least one black colorant and one or more external additives, wherein the toner particles comprise from about 7 to about 15 pph of the developer, and wherein the toner particles exhibit a triboelectric charge of from about -25 to about -50  $\mu$ C/g at toner particle concentrations of about 7 to about 15 pph of the developer. The developer is ideally suited for use in a high speed (greater than 100 prints per minute) semiconductive magnetic brush development apparatus. Preferably, the black toner particles include a styrene acrylate binder, and the external additives include from about 1.3 to about 2.1% by weight of the toner particles of a first silica having an average particle size of from about 35 to about 45 nm, from about 0.5 to about 1.0% by weight of the toner particles of a second silica having an average particle size of from about 135 to about 160 nm, and from about 0.2 to about 0.5% by weight of the toner particles of a titania having an average particle size of from about 35 to about 45 nm, with an external additive toner surface area coverage of from about 25 to about 45%.

**19 Claims, No Drawings**

## 1

## BLACK TONER AND DEVELOPER

CROSS-REFERENCE TO RELATED  
APPLICATION

This application is a continuation-in-part application of U.S. application Ser. No. 10/839,293 filed May 6, 2004, now U.S. Pat. No. 7,157,200 which application is incorporated by reference herein in its entirety.

## BACKGROUND

Described herein are black toners, developers containing the black toners, and a method of forming images with the developers, preferably utilizing a semiconductive magnetic brush development system. More in particular, described herein are black toners having specific properties and/or compositions such that the toner, following triboelectric contact with a carrier, exhibits a triboelectric charge of from about -25 to about -50  $\mu\text{C/g}$  so as to provide a black toner image of superior image quality when used to develop electrostatic images, particularly in a semiconductive magnetic brush development system.

U.S. Pat. No. 5,545,501 describes an electrostatographic developer composition comprising carrier particles and toner particles with a toner particle size distribution having a volume average particle size ( $t$ ) (such that  $4 \mu\text{m} \leq t \leq 12 \mu\text{m}$  and an average charge (absolute value) per diameter in femtocoulomb/10  $\mu\text{m}$  ( $C_T$ ) after triboelectric contact with said carrier particles such that  $1 \text{fc}/10 \mu\text{m} \leq C_T \leq 10 \text{fc}/10 \mu\text{m}$  characterized in that (i) said carrier particles have a saturation magnetization value,  $M_{sat}$ , expressed in Tesla (T) such that  $M_{sat} \geq 0.30 \text{ T}$ , (ii) said carrier particles have a volume average particle size ( $C_{avg}$ ) such that  $30 \mu\text{m} \leq C_{avg} \leq 60 \mu\text{m}$ , (iii) said volume based particle size distribution of said carrier particles has at least 90% of the particles having a particle diameter  $C$  such that  $0.5 C_{avg} \leq C \leq 2 C_{avg}$ , (iv) said volume based particles size distribution of said carrier particles comprises less than  $b$  % particles smaller than  $25 \mu\text{m}$  wherein  $b = 0.35 \times (M_{sat})^2 \times P$  with  $M_{sat}$ =saturation magnetization value,  $M_{sat}$ , expressed in T and P=the maximal field strength of the magnetic developing pole expressed in kA/m, and (v) said carrier particles comprise a core particle coated with a resin coating in an amount (RC) such that  $0.2\% \text{ w/w} \leq RC \leq 2\% \text{ w/w}$ . See the Abstract. This patent describes that such developer achieves images of offset-quality in systems in which a latent image is developed with a fine hair magnetic brush. See column 4, lines 7-17 of the patent.

U.S. Pat. No. 6,319,647 describes a toner of toner particles containing at least one binder, at least one colorant, and preferably one or more external additives that is advantageously formed into a developer and used in a magnetic brush development system to achieve consistent, high quality copy images. The toner particles, following triboelectric contact with carrier particles, exhibit a charge per particle diameter (Q/D) of from 0.6 to 0.9  $\text{fC}/\mu\text{m}$  and a triboelectric charge of from 20 to 25  $\mu\text{C/g}$ . The toner particles preferably have an average particle diameter of from 7.8 to 8.3 microns. The toner is combined with carrier particles to achieve a developer, the carrier particles preferably having an average diameter of from 45 to 55 microns and including a core of ferrite substantially free of copper and zinc coated with a coating comprising a polyvinylidenefluoride polymer or copolymer and a polymethyl methacrylate polymer or copolymer.

## 2

U.S. Pat. No. 6,361,915 describes a process for manufacturing a conductive micropowder and includes the steps of: (i) forming an aqueous dispersion of conductive material and the first surfactant, (ii) mixing a latex emulsion of a polymer and a second surfactant into the aqueous dispersion to form a suspension and (iii) recovering the conductive micropowder from the suspension. The first and second surfactants are of the same class and polarity. The conductive micropowder finds particular utility as a coating for carrier core particles, and as a conductive coating component of carrier particle coatings.

U.S. Pat. No. 6,416,916 describes a toner of toner particles containing at least one binder, at least one colorant, and an external additive package comprised of zinc stearate and at least one of silicon dioxide or titanium dioxide, wherein the amount of zinc stearate is limited to about 0.10 percent by weight or less of the toner. It is reported that when the amount of zinc stearate is so limited, a developer formed from the toner exhibits excellent triboelectric charging and stability and excellent developer flow. When the developer is used in a magnetic brush development system, consistent, high quality copy images are formed substantially without any depletion defects over time.

What is still desired is a black toner for use in semiconductive magnetic brush development systems, which toner is able to develop a large number of pages per minute having high image density with substantially reduced emissions and high print quality.

## SUMMARY

In embodiments, described are developers comprised of toner particles of at least one binder, at least one black colorant and one or more external additives, together with carrier particles, wherein the toner particles comprise from about 7 to about 15 pph of the developer, and wherein the toner particles exhibit a triboelectric charge of from about -25 to about -50  $\mu\text{C/g}$  at toner particle concentrations of about 7 to about 15 pph of the developer.

In embodiments, the toner particles include from about 6 to about 10% by weight of the black colorant, and the developer provides a solid area image density of from about 19 to about 23 at a transferred toner mass per area of about 0.35 to about 0.55  $\text{mg/cm}^2$ .

In embodiments, the black toner particles comprise at least one binder, at least one black colorant, and external additives, wherein the at least one binder includes a styrene acrylate binder including a cross-linked styrene acrylate gel content of from 0% to about 12% by weight of the binder, wherein the external additives include from about 1.3 to about 2.1% by weight of the toner particles of a first silica having an average particle size of from about 35 to about 45 nm, from about 0.5 to about 1.0% by weight of the toner particles of a second silica having an average particle size of from about 135 to about 160 nm, and from about 0.2 to about 0.5% by weight of the toner particles of a titania having an average particle size of from about 35 to about 45 nm, and wherein the external additives have a toner surface area coverage of from about 25 to about 45%.

In further embodiments, the styrene acrylate binder is comprised of a copolymer of styrene, n-butyl acrylate and  $\beta$ -carboxyethyl acrylate, preferably of from about 70 to about 90% by weight styrene, about 10 to about 30% by weight n-butyl acrylate and about 0.5 to about 10 pph of the binder of  $\beta$ -carboxyethyl acrylate.

In still further embodiments, the carrier particles of the developer comprise a core, preferably of ferrite, coated with

a coating comprising a polymethyl methacrylate polymer or copolymer, fluorine-containing polymer or copolymer, carbon black and melamine beads, preferably including about 73 to about 77% by weight of the coating of the polymethyl methacrylate polymer or copolymer, about 5 to about 7% by weight of the fluorine-containing polymer or copolymer, about 8 to about 10% by weight carbon black and about 9 to about 11% by weight of the melamine beads. Preferably the polymethyl methacrylate polymer or copolymer is prepared as a latex using sodium lauryl sulfate (SLS) as the surfactant in the latex preparation step, followed by drying of the latex prior to coating the carrier core. Preferably, the coating is present in an amount of about 0.6 to about 1.0% by weight of the carrier.

In still further embodiments, described is an electrophotographic image forming apparatus comprising a photoreceptor, a semiconductive magnetic brush development system, and a housing in association with the semiconductive magnetic brush development system for containing the developers described herein.

#### DETAILED DESCRIPTION OF EMBODIMENTS

Generally, the process of electrophotographic printing includes charging a photoconductive member to a substantially uniform potential to sensitize the surface thereof. The charged portion of the photoconductive surface is exposed to a light image from, for example, a scanning laser beam, an LED source, etc., and of an original document being reproduced. This records an electrostatic latent image on the photoconductive surface of a photoreceptor. After the electrostatic latent image is recorded on the photoconductive surface, the latent image is developed with a toner or developer containing a toner.

A two-component developer is used herein for development. A typical two-component developer comprises magnetic carrier particles with toner particles triboelectrically attracted thereto. During development of the latent image, the toner particles are attracted to the latent image, forming a toner powder image on the photoconductive surface. The toner powder image is subsequently transferred to an image transfer medium, e.g., a sheet of paper or a transparency, either directly or via an intermediate transfer member. Finally, the toner powder image is heated to permanently fuse it to the image transfer medium.

A commonly known way of developing the latent image on the photoreceptor is by use of one or more magnetic brushes. See, for example, U.S. Pat. Nos. 5,416,566, 5,345, 298, 4,465,730, 4,155,329 and 3,981,272, incorporated herein by reference. The toner of the developer may be formulated to carry either a negative or positive charge, and is in any case selected vis-a-vis the carrier so that the toner particles acquire the proper operating charge with respect to the latent electrostatic image being developed. Thus, when the developer is brought into operative contact with the photoconductive surface of the photoreceptor, the greater attractive force of the discharged image causes the toner particles to leave the carrier particles and adhere to the image portion of the photoconductive surface.

The previously mentioned magnetic brush typically is comprised of a roll having a tube-like member or sleeve, which is rotatably supported. The sleeve is preferably made from a non-magnetic material, more preferably stainless steel, which is conductive and allows less eddy currents than aluminum so that localized heating is reduced. One or more magnets are mounted inside the sleeve. The roll is disposed

so that a portion of the sleeve is immersed in or in contact with a supply of developer comprising the carrier particles and the toner particles.

As a result, the developer is made to be attracted to the surface of the sleeve and arranges thereupon in the form of a brush, e.g., as bristles of a brush. Thus, when the photoreceptor bearing the latent electrostatic image thereon is brought into physical contact with the brush, the attractive force of the electrostatic charge on the photoreceptor surface in the image areas, which is greater than the force holding the toner particles in association with the brush, draws the toner particles from the magnetic brush roller and onto the image areas to render the image visible.

The electrophotographic marking process given above is ideal for single color images, i.e., conventional black toner images. In such process, the toner particles are colored black by way of a black colorant included in the toner particles.

Described herein are novel developers including black toner that operate in the restrictive semiconductive magnetic brush development environment to achieve image qualities superior to prior art toners and developers with the capability of forming a large number of prints per minute (e.g., 100 or more prints per minute) with reduced emissions and excellent background performance. As a result of the reduced emissions with the toner, solid and halftone areas are uniform and stable in density and color, and text is crisp with well-defined edges regardless of font size or type. In addition, background toner in non-image areas is reduced, in particular to less than 100 particles per  $\text{mm}^2$ , preferably less than 50 particles per  $\text{mm}^2$ , and machine dirt and contamination is minimized.

In embodiments, the developer comprises black toner particles and carrier particles, wherein the black toner particles comprise at least one binder, at least one black colorant and one or more external additives, wherein the toner particles comprise from about 7 to about 15 pph of the developer, and wherein the toner particles exhibit a triboelectric charge of from about -25 to about -50  $\mu\text{C/g}$  at toner particle concentrations of about 7 to about 15 pph of the developer.

This triboelectric charging versus toner concentration has been found to permit the preferred high speed semiconductive magnetic brush development system to operate with the aforementioned minimal background and substantially no dirt or contamination. Moreover, the developer is able to provide a solid area image density of from about 19 to about 23 at a transferred toner mass per area of about 0.35 to about 0.55  $\text{mg/cm}^2$ . Solid area image density as described herein is measured with a Gretag Macbeth reflection spectrodensitometer or other suitable and/or similar device. It has further been found that in achieving the aforementioned developer properties, it is desirable that the toner particles include from about 6 to about 10% by weight of the black colorant, most preferably carbon black. The minimum black colorant loading of about 6% by weight of the toner has been found necessary in embodiments in order to achieve the desired solid image area density, and the maximum loading amount of about 10% by weight of the toner black colorant has been found necessary in embodiments to limit the background to acceptable levels.

The black toner is preferably comprised of at least one resin binder, at least one black colorant and an external additive package comprised of one or more particulate additives. Suitable and preferred materials for use in preparing the black toner are discussed below.

In the black toner, the resin binder of the toner particles is preferably comprised of an acrylate binder, more prefer-

ably a styrene acrylate binder, most preferably of an emulsion aggregation styrene acrylate binder.

If an emulsion aggregation styrene acrylate binder is used, such may be prepared by any suitable emulsion aggregation process. As one example, reference is made to U.S. Pat. No. 6,120,967, incorporated herein by reference in its entirety. Emulsion aggregation is a chemical process of forming the toner particles, wherein the toner particles are built up from an emulsion of the toner particle materials. Such a chemical process is generally preferred over conventional physical processes that require grinding and sizing to achieve the desired toner particle size and size distribution.

In embodiments, the styrene acrylate binder of the toner particles is comprised of a copolymer of at least styrene, n-butyl acrylate and  $\beta$ -carboxyethyl acrylate. Preferably, the copolymer is derived from about 70 to about 90% by weight of the copolymer of styrene, about 10 to about 30% by weight n-butyl acrylate and about 0.5 to about 10 pph of the binder of  $\beta$ -carboxyethyl acrylate, and more preferably about 15 to 25% by weight n-butyl acrylate and about 1 to about 6 pph of the binder of  $\beta$ -carboxyethyl acrylate.

The styrene acrylate binder may be made to include some amount of cross-linked gel portions therein. These cross-linked gel portions are comprised of cross-linked binder distributed as microgel particles throughout the linear portions of the binder. Such cross-linked gel portions have a volume average particle size of from, for example, 0.1  $\mu$ m or less, preferably about 0.005 to about 0.1  $\mu$ m, as determined by scanning electron microscopy and/or transmission electron microscopy.

The binder resin preferably has a weight fraction of the microgel (cross-linked gel portion content) in the range from 0 to about 15% by weight of the binder, preferably from about 0 to about 12% by weight of the binder, more preferably from about 6 to about 12% by weight of the binder. The linear portion is comprised of base resin, preferably styrene acrylate, in the range from about 50 to about 100% by weight of the binder, and preferably in the range from about 65 to about 100% by weight of the binder. The linear portion of the binder resin preferably comprises low molecular weight reactive base resin that did not cross-link during a cross-linking reaction. The molecular weight distribution of the styrene acrylate binder resin is thus bimodal, having different ranges for the linear and the cross-linked portions of the binder resin.

The binder may also include some amount of additional binder materials such as comprised of, for example, vinyl polymers such as styrene polymers, acrylonitrile polymers, vinyl ether polymers, acrylate and methacrylate polymers; epoxy polymers; diolefins; polyurethanes; polyamides and polyimides; polyesters such as the polymeric esterification products of a dicarboxylic acid and a diol comprising a diphenol, crosslinked polyesters; and the like.

The binder of the toner particles is melt blended or otherwise mixed with at least one black colorant. Various black colorants may be used without limitation, and the colorant may be a pigment, dye or mixture thereof. Example black colorants include, for example, carbon black such as REGAL 330 carbon black (Cabot), acetylene black, lamp black, aniline black and mixtures thereof. Most preferably, the colorant is a carbon black pigment having a suitable particle size such as, for example, about 50 to about 250 nm, and may be in the form of a dispersion, for example an aqueous dispersion.

The black colorant is preferably included in the toner composition in an amount of from about 1% to about 25% by weight of the toner particles, preferably from about 5%

to about 15% by weight of the toner particles, most preferably from about 6 to about 10% by weight of the toner particles, as discussed above.

The toner particles may also include several additional optional additives within the toner particles (e.g., internal additives). For example, as required, the toner particles may also include charge control additives, surfactants, emulsifiers, pigment dispersants, flow additives, and the like.

A wax, such as polyethylene, polypropylene, and/or paraffin wax, is also preferably included in or on the toner composition as a fusing release agent. In embodiments, the wax is included in the toner particles in an amount of from about 5 to about 15% by weight of the toner particles.

The toner particles of the present invention preferably have a small size. In particular, the toner particles preferably have an average particle size of from about 3  $\mu$ m to about 10  $\mu$ m, preferably from about 4  $\mu$ m to about 7  $\mu$ m, most preferably from about 5  $\mu$ m to about 6  $\mu$ m.

The toner particles also have one or more external additives on the surface of the toner particles.

Preferably, the external additives comprise at least a first silica having an average particle size of from about 35 to about 45 nm, a second silica having an average particle size of from about 135 to about 160 nm, and a titania having an average particle size of from about 35 to about 45 nm.

The first silica (also known as  $\text{SiO}_2$  or silicon dioxide) is preferably present in the toner particles in an amount of from about 1.0 to about 3.0% by weight of the toner particles, preferably from about 1.3 to about 2.1% by weight of the toner particles. This first silica particle preferably has an average particle size of about 40 nm. In general, silica is applied to the toner surface for toner flow, triboelectric enhancement, admix control, improved development and transfer stability and higher toner blocking temperature. It has been found that the aforementioned amounts of the sized first silica in the toner particles can increase the toner particles triboelectric charge in use and can also increase the charge per particle diameter (q/d) of the toner in use. Silica particles of the aforementioned size range are commercially available, for example from Nippon Aerosil Co., (NAC), Tokyo, Japan.

The second silica is preferably present in the toner particles in an amount of from about 0.2 to about 2.0% by weight of the toner particles, preferably from about 0.5 to about 1.0% by weight of the toner particles. This second silica particle preferably has an average particle size of about 140 nm to about 150 nm. It has been found that this second silica may increase the cohesion of the toner particles, but not to an extent that is unacceptable within the aforementioned amount ranges. The second silica does not negatively affect the triboelectric charging or q/d properties of the toner particles.

The presence of these ultra large size second silica particles is desirable in order to prevent impaction of the smaller sized external additives into the toner particles during use of the toner. During use, carrier particles knock into the toner particles, and such impacts can force smaller external additives to become undesirably impacted into the surface of the toner particles. The larger sized second silica particles absorb the impacts, and are of a sufficiently large size themselves to be less susceptible to complete impaction into the toner particles. The presence of the second silica particles thus ensures maintained development and transfer performance of the toner over time.

The second silica particles are preferably sol-gel silica particles. The second silica particles are commercially available, for example from Shin-Etsu.

The titania particles (also known as  $\text{TiO}_2$  or titanium dioxide) is preferably present in the toner particles in an amount of from about 0.1 to about 1.0% by weight of the toner particles, preferably from about 0.2 to about 0.5% by weight of the toner particles. This titania particles preferably have an average particle size of about 40 nm. In general, titania is added to the surface of the toner particles for improved relative humidity (RH) stability, triboelectric control and improved development and transfer stability. Titania particles of the aforementioned size range are commercially available, for example from Tayca.

Optionally, a third silica may be present in the toner particles in an amount of from about 0.2 to about 5.0% by weight of the toner particles. This third silica particle preferably has an average particle size of about 8 nm to about 20 nm. The third silica may contribute to improved charging and flowability. Example suitable silicas in the size range of 8 nm to 20 nm and are commercially available from Degussa and Cabot Corporation.

The external additives preferably are provided on the surface of the toner particles in an amount such that the external additives have a toner surface area coverage (SAC) of from about 25 to about 95%, preferably at least about 25 to about 45%. Developer life can increase with higher SAC for high printing systems.

Additional external surface additives may also be included in the external surface additive package. For example, the external additive package may also include ZnSt (zinc stearate). Zinc stearate provides lubricating properties, provides developer conductivity and triboelectric enhancement, both due to its lubricating nature, and can enable higher toner charge and charge stability by increasing the number of contacts between toner and carrier particles. Calcium stearate and magnesium stearate may also be added to provide similar functions. A suitable commercially available zinc stearate is known as Zinc Stearate L made by Ferro Corporation, Polymer Additives Division.

The aforementioned external additives may be rendered hydrophobic, if necessary, by surface treatments to reduce the humidity sensitivity of the toner charging. The first silica and titania, for example, may be treated with PDMS (polydimethyl siloxane). The second silica may be treated with, for example, an organic lane.

The following Table 1 sets forth several preferred toner compositions, in which in Examples 1-8 preferred upper and lower limits of the external additives are used and in Example 9 a middle value for each component is used. All amounts are percentages by weight, based on the total weight of the toner particles.

TABLE 1

| Example | First small size silica | Second large size silica | Titania |
|---------|-------------------------|--------------------------|---------|
| 1       | 1.37                    | 0.59                     | 0.30    |
| 2       | 2.05                    | 0.59                     | 0.30    |
| 3       | 1.37                    | 0.89                     | 0.30    |
| 4       | 2.05                    | 0.89                     | 0.30    |
| 5       | 1.37                    | 0.59                     | 0.44    |
| 6       | 2.05                    | 0.59                     | 0.44    |
| 7       | 1.37                    | 0.89                     | 0.44    |
| 8       | 2.05                    | 0.89                     | 0.44    |
| 9       | 1.71                    | 0.74                     | 0.37    |

The toner composition can be prepared by a number of known methods, for example including physical methods such as melt blending the toner resin particles, colorants and optional internal additives followed by mechanical attrition. The toner may be made by first mixing the binder, preferably

comprised of both the linear resin and the cross-linked resin as discussed above, and the colorant, along with optional additives including a wax, together in a mixing device. The toner is then classified to form a toner with the desired volume median particle size. Care should be taken in the method in order to limit the coarse particles, grits and giant particles. Subsequent toner blending of the external additives is preferably accomplished using a mixer or blender, for example a Henschel mixer, followed by screening to obtain the final toner product.

Other methods include those well known in the art such as spray drying, melt dispersion, dispersion polymerization, suspension polymerization, emulsion aggregation and extrusion. In embodiments, the toner particles are preferably formed via a chemical method, in particular emulsion aggregation. For example, such a process may include at least forming a latex dispersion of the toner binder materials, preparing a pigment dispersion, blending the latex dispersion with the pigment dispersion, and optionally a wax dispersion, to form a resin-pigment blend, adding a coagulant to the resin-pigment blend, while continuously subjecting the mixture to high shear, preferably with heating below a glass transition temperature ( $T_g$ ) of the resin binder, to form aggregate particles, and heating the aggregate particles at temperatures above the  $T_g$  of the binder resin, optionally with reduction of the pH, to form coalesced toner particles.

Following formation via emulsion aggregation, the toner particles may optionally be washed with an acid, e.g., calcium chloride. Such acid washing can improve the relative humidity sensitivity of the toner particles but can also lower triboelectric charging values of the toner particles. Water washing, which does not substantially affect the toner particle properties, may alternatively be used.

The charge of a toner is described in terms of the charge/particle diameter,  $q/d$ , in  $\text{fC}/\mu\text{m}$  following triboelectric contact of the toner with carrier particles. The charge per particle diameter ( $q/d$ ) of the toner particles preferably has an average value of from, for example,  $-0.1$  to  $-1.5 \text{ fC}/\mu\text{m}$ . This charge should remain stable throughout the development process in order to insure consistency in the richness of the images obtained using the toner. The measurement of the average  $q/d$  of the toner particles can be done by means of a charge spectrograph apparatus as well known in the art. See, for example, U.S. Pat. No. 4,375,673, incorporated herein by reference. The spectrograph is used to measure the distribution of the toner particle charge ( $q$  in  $\text{fC}$ ) with respect to a measured toner diameter ( $d$  in  $\mu\text{m}$ ).

In a most preferred embodiment of the present invention, the toner particles exhibit a triboelectric value (as measured by the known blowoff process using a Faraday Cage), after triboelectric contact with carrier particles, of from, for example, about  $-25$  to about  $-50 \mu\text{C}/\text{g}$ , as measured in  $70^\circ \text{ F}$ . and 50% relative humidity, as well as exhibits triboelectric stability over the life of the developer.

The toner is most preferably incorporated into a two component developer composition as discussed above by mixing with appropriate carrier particles.

Suitable and preferred materials for use as carriers used in preparing developers containing the above-discussed toners that possess the properties discussed above will now be discussed. The toner particles triboelectrically associate and/or adhere to the surface of the carrier particles.

Illustrative examples of carrier particles that can be selected for mixing with the toner composition prepared in accordance with the present invention include those particles that are capable of triboelectrically obtaining a charge of opposite polarity to that of the toner particles. Illustrative

examples of suitable carrier particles include granular zircon, granular silicon, glass, steel, nickel, ferrites, iron ferrites, silicon dioxide, and the like. Other suitable carriers are disclosed in U.S. Pat. Nos. 4,937,166 and 4,935,326, the disclosures of which are hereby totally incorporated by reference.

In a preferred embodiment, the carrier core is comprised of ferrite particles. Any commercially available ferrite carrier may be used without restriction. Preferably, the carrier core may be comprised of a manganese magnesium ferrite core, such as commercially available from Powder Tech. The ferrite particles to be used as carrier cores in the developer composition preferably have an average particle size (diameter) of from, for example, 10 to 100  $\mu\text{m}$ , preferably 20 to 70  $\mu\text{m}$ , most preferably 25 to 40  $\mu\text{m}$ , as determined by standard laser diffraction techniques.

The selected carrier particles can be used with or without a coating. In a preferred embodiment of the developer composition, the carrier particles are coated with a polymethyl methacrylate polymer or copolymer.

In another preferred embodiment, the ferrite carrier particles are coated with a mixture of at least two dry polymer components, which dry polymer components are preferably not in close proximity thereto in the triboelectric series, and most preferably of opposite charging polarities with respect to the toner selected. The electronegative polymer, i.e., the polymer that will generally impart a negative charge on the toner with which it is contacted, is preferably comprised of a fluorine-containing polymer or copolymer, e.g., polyvinylidenefluoride polymer or copolymer. Such polyvinylidenefluoride polymers are commercially available, for example under the tradename KYNAR. The electropositive polymer, i.e., the polymer that will generally impart a negative charge on the toner with which it is contacted, is preferably comprised of a polymer or copolymer of polymethyl methacrylate (PMMA), optionally having carbon black or another conductive material dispersed therein. PMMA by itself is an insulative polymer. To obtain a conductive carrier coating, a conductive component, for example carbon black, is dry blended with the PMMA and any other carrier coating constituents. The mixture is then tumbled onto the core and fused.

The PMMA may be copolymerized with any desired comonomer, so long as the resulting copolymer retains a suitable particle size. Suitable comonomers can include monoalkyl, or dialkyl amines, such as a dimethylaminoethyl methacrylate, diethylaminoethyl methacrylate, diisopropylaminoethyl methacrylate, t-butylaminoethyl methacrylate, and the like. If the PMMA polymer has carbon black dispersed therein, it is preferably formed in a semisuspension polymerization process, for example as described in U.S. Pat. No. 5,236,629, incorporated by reference herein in its entirety.

In a preferred embodiment of the invention, the carrier is coated with a PMMA coating such as described in U.S. Pat. No. 5,847,030, incorporated herein by reference in its entirety. Preferably, such PMMA is made by an emulsion polymerization process and has a narrow particle size distribution with polymer particles in the 100 to 200 nm size range, preferably about 150 nm. This small size is desirable to provide uniform coverage on the small ferrite core. It is further preferred that the polymethyl methacrylate prepared by emulsion polymerization is prepared in the presence of sodium lauryl sulphate surfactant to form the latex.

The percentage of each polymer present in the carrier coating can vary depending on the specific components selected, the coating weight and the properties desired. For

example, the ratios of the two polymers may be varied in order to adjust the triboelectric characteristics of the carrier in order to meet the particular requirements of a given printing device. Generally, the coated polymer mixtures used contain from about 3 to about 97 percent of the electronegative polymer, and from about 97 to about 3 percent by weight of the electropositive polymer. Preferably, there are selected mixtures of polymers with from about 3 to 25 percent by weight of the electronegative polymer, and from about 97 to 75 percent by weight of the electropositive polymer. Most preferably, there are selected mixtures of polymers with from about 5 to 15 percent by weight of the electronegative polymer, and from about 95 to 85 percent by weight of the electropositive polymer.

In a most preferred embodiment, the coating on the carrier particles includes from about 70 to about 80% by weight, preferably about 73 to about 77% by weight, of a polymethyl methacrylate polymer or copolymer, from about 6 to about 12% by weight, preferably about 8 to about 10% by weight, of carbon black, from about 8 to about 12% by weight, preferably from about 9 to about 11% by weight, of melamine beads, and from about 3 to about 10% by weight, preferably about 5 to about 7% by weight, of a fluorine-containing polymer or copolymer.

As noted above, the coating on the ferrite carrier particles preferably also includes melamine beads, for example melamine beads having an average particles size of from about 100 nm to about 300 nm. Such beads are commercially available from, for example, Nippon Shokubai. The melamine beads may comprise of from about 5 to about 15% by weight of the total coating, more preferably from about 8 to about 12% by weight of the total coating. The melamine beads may provide charging and conductivity stability.

The carrier particles may be prepared by mixing the carrier core with from, for example, between about 0.05 to about 10 percent by weight, most preferably between about 0.3 percent and about 5.0 percent by weight, based on the weight of the coated carrier particles, of the coating composition until adherence thereof to the carrier core by mechanical impaction and/or electrostatic attraction. The mixture of carrier core particles and polymers is then heated to an elevated temperature for a period of time sufficient to melt and fuse to the coating polymers to the carrier core particles. The coated carrier particles are then cooled and thereafter classified to a desired particle size. The coating preferably has a coating weight of from, for example, 0.1 to 5.0% by weight of the carrier, preferably 0.6 to 1.0% by weight.

Various effective suitable methods can be used to apply the polymer mixture coatings to the surface of the carrier core particles. Examples of typical methods for this purpose include combining the carrier core material and the coating composition by cascade roll mixing, or tumbling, milling, shaking, electrostatic powder cloud spraying, fluidized bed, electrostatic disc processing, and an electrostatic curtain.

The coated carrier particles preferably have a size of from about 25  $\mu\text{m}$  to about 40  $\mu\text{m}$ , more preferably of about 35  $\mu\text{m}$ . In a preferred embodiment, it is desirable to maintain a ratio of carrier volume median diameter to toner volume median diameter of approximately 5:1 to 9:1.

Two component developer compositions of the present invention can be generated by mixing the carrier core particles with the toner composition discussed above. The carrier particles can be mixed with the toner particles in various suitable combinations. However, best results are obtained when from about 1 part to about 25 parts by weight of the black toner and from about 75 parts to about 99 parts

## 11

by weight of the carrier particles, are mixed. Preferably, the toner concentration in the developer is from about 7 to about 15 pph of the developer. The toner concentration in the developer initially installed in a xerographic development housing is thus preferably between, for example, about 7 to about 15% by weight based on the total developer weight.

The developers of the invention exhibit superior black image quality, reduced emissions, and enable the device to print a large number of pages per minute (ppm), for example on the order of 100 to 200 ppm or more, without quality problems arising.

To determine the tribo, a 0.5 gram sample of developer is placed in a Faraday cage. Pressurized air is blown through the cage that has screens at each end. The screen size allows toner to escape and retains carrier. A 15 micron screen is best for 35 micron carrier and 5.5 micron toner. An electrometer is attached to the cage and monitors charge change as toner exits the cage. The weight change is measured from before to after blowoff and toner mass is obtained. Tribo is defined as toner charge/toner mass. Developability may fall off if toner surface additives move to the carrier, if the surface additives get impacted into the toner and or if the developer conductivity drops.

The measured background for each of the Example toners 1-9 above is very low, and is below about 50 particles per mm<sup>2</sup>. Background is measured by picking up untransferred toner off the photoreceptor with adhesive tape and counting the number of toner particles per square millimeter.

While the subject matter has been described in conjunction with specific embodiments described above, it is evident that many alternatives, modifications and variations will be apparent to those skilled in the art. Accordingly, the embodiments, as set forth above, are intended to be illustrative and not limiting. Various changes may be made without departing from the spirit and scope of the subject matter described herein.

What is claimed is:

1. A developer comprising black toner particles and carrier particles, wherein the black toner particles comprise at least one binder, at least one black colorant and one or more external additives, wherein the toner particles comprise from about 7 to about 15 pph by weight of the developer, and wherein the toner particles exhibit a triboelectric charge of from about -25 to about -50  $\mu$ C/g at toner particle concentrations of about 7 to about 15 pph by weight of the developer.

2. The developer according to claim 1, wherein the toner particles include from about 6 to about 10% by weight of the black colorant.

3. The developer according to claim 1, wherein the developer provides a solid area image density of from about 19 to about 23 at a transferred toner mass per area of about 0.35 to about 0.55 mg/cm<sup>2</sup>.

4. The developer according to claim 1, wherein the developer provides a background of less than 100 particles/mm<sup>2</sup>.

5. The developer according to claim 1, wherein the toner particles are emulsion aggregation toner particles.

6. A developer comprising black toner particles and carrier particles, wherein the black toner particles comprise at least one binder, at least one black colorant, and external additives, wherein the at least one binder includes a styrene acrylate binder including a cross-linked styrene acrylate gel content of from 0% to about 12% by weight of the binder, wherein the external additives include from about 1.3 to about 2.1% by weight of the toner particles of a first silica having an average particle size of from about 35 to about 45

## 12

nm, from about 0.5 to about 1.0% by weight of the toner particles of a second silica having an average particle size of from about 135 to about 160 nm, and from about 0.2 to about 0.5% by weight of the toner particles of a titania having an average particle size of from about 35 to about 45 nm, and wherein the external additives have a toner surface area coverage of from about 25 to about 45%.

7. The developer according to claim 6, wherein the toner particles comprise from about 7 to about 15 pph by weight of the developer.

8. The developer according to claim 6, wherein the carrier particles comprise a core of ferrite coated with a coating comprising a polymethyl methacrylate polymer or copolymer, a fluorine-containing polymer or copolymer, carbon black and melamine beads.

9. The developer according to claim 8, wherein the coating comprises from about 73 to about 77% by weight of the coating of the polymethyl methacrylate polymer or copolymer, from about 5 to about 7% by weight of the coating of the fluorine-containing polymer or copolymer, from about 8 to about 10% by weight of the coating of the carbon black and from about 9 to about 11% by weight of the coating of the melamine beads.

10. The developer according to claim 8, wherein the coating is present in an amount of about 0.6 to about 1.0% by weight of the carrier.

11. The developer according to claim 6, wherein the cross-linked styrene acrylate gel content of the toner particles is from 6% to about 12% by weight of the binder.

12. The developer according to claim 6, wherein the styrene acrylate binder of the toner particles is comprised of a copolymer of styrene, n-butyl acrylate and  $\beta$ -carboxyethyl acrylate.

13. The developer according to claim 12, wherein the copolymer is derived from about 70 to about 90% by weight styrene, about 10 to about 30% by weight n-butyl acrylate and about 0.5 to about 10 pph by weight of the binder of  $\beta$ -carboxyethyl acrylate.

14. The developer according to claim 6, wherein the at least one black colorant includes carbon black.

15. The developer according to claim 6, wherein the second silica is a sol-gel silica.

16. The developer according to claim 6, wherein the toner particles further comprise from about 5 to about 15% by weight of the toner particles of a wax.

17. The developer according to claim 6, wherein the toner particles have an average particle size of from about 4 to about 7  $\mu$ m.

18. The developer according to claim 6, wherein the carrier particles have an average diameter of from about 30 to about 55  $\mu$ m.

19. An electrophotographic image forming apparatus comprising a photoreceptor, a semiconductive magnetic brush development system, and a housing in association with the semiconductive magnetic brush development system, wherein the housing delivers to the semiconductive magnetic brush development system a developer comprising black toner particles and carrier particles, wherein the black toner particles comprise at least one binder, at least one black colorant and one or more external additives, wherein the toner particles comprise from about 7 to about 15 pph by weight of the developer, and wherein the toner particles exhibit a triboelectric charge of from about -25 to about -50  $\mu$ C/g at toner particle concentrations of about 7 to about 15 pph by weight of the developer.

UNITED STATES PATENT AND TRADEMARK OFFICE  
**CERTIFICATE OF CORRECTION**

PATENT NO. : 7,309,556 B2  
APPLICATION NO. : 11/083934  
DATED : December 18, 2007  
INVENTOR(S) : Vladislav Skororkhod et al.

Page 1 of 1

It is certified that error appears in the above-identified patent and that said Letters Patent is hereby corrected as shown below:

Item (12), line 2:

Please change "Mc Dougall" to read --McDougall--

Item (75), line 1:

Please change "Mc Dougall" to read --McDougall--

Item (75), line 5:

Please change "Mc Stravick" to read --McStravick--

Item (75), line 8:

Please change "Mc Grath" to read --McGrath--.

Signed and Sealed this

Nineteenth Day of February, 2008



JON W. DUDAS  
*Director of the United States Patent and Trademark Office*